

## UNITED STATES PATENT OFFICE

ALEXANDER L. ULLRICH, OF CHICAGO, ILLINOIS

## PROCESS OF MANUFACTURING AMORPHOUS CARBON

No Drawing.

Application filed April 24, 1925. Serial No. 25,619.

My invention in general relates to a process of manufacturing amorphous carbon, and more particularly to a process of manufacturing lamp black from tar. Still more specifically, the invention has reference to the manufacture of lamp black from high carbon tar or tar having constituents belonging to the class of "aromatic" hydrocarbons, such as coal tar and water gas tar.

Now, it is well known to those familiar with the present art, that lamp black, which is a deep black pigment consisting of carbon in a very fine state of division, is obtained commercially by the imperfect combustion of highly carbonaceous substances such as from scraps of rosin and pitch, inferior oils, fats and other similar combustible matter rich in carbon. The finest lamp black, however, is procured by the combustion of oil, obtained in coal tar distillation.

The principal aim or proposal of the present invention, is to manufacture amorphous carbon, such as lamp black, directly from coal tar, in a much more economical manner than any of the heretofore methods of manufacturing lamp black.

I am aware that lamp black has also heretofore been manufactured by burning tar in ovens connected with brick chambers in which large quantities of soot formed in this process, deposit before the gases escape through the chimney. This method of manufacture is far more expensive than my improved method, to be hereinafter described. Then, too, this manner of procuring lamp black by the incomplete combustion of carbonaceous matter results in noxious gases being evolved which usually are permitted to escape into the atmosphere thereby fouling the air of the community. My proposed improved method of manufacturing lamp black does not require the combustion of any carbonaceous matter, and hence, no noxious gases are generated. Also, more carbon of the above character can be obtained by my improved process from a predetermined quantity of tar than any other method or process that I am aware of.

The primary object therefore of the present invention, is to provide an improved

method of manufacturing amorphous carbon, such as lamp black, from high carbon tars.

Other objects and advantages of the present invention will more fully appear from the following description of the method.

The first step involved, is to bring the tar to a liquid form. As previously mentioned, the tar is one having a relatively great amount of carbon therein. I prefer to use a coal tar or a water gas tar. Liquefaction of the tar is carried out by heating the tar. The tar may be placed in any suitable receptacle and heated in any desirable or convenient manner.

I find it desirable to add a solvent to the liquid tar. The solvent employed may be benzol, amyl acetate, or any solvent of a like or suitable character. In carrying out my process benzol was used as the solvent, due to its being a very cheap and easy one to procure.

The solvent, when added at this stage of the process, seems to aid in the liquefying of the coal tar. The solvent added may be equal in volume to the coal tar being heated. That is to say, if one gallon of tar is heated, a gallon of solvent is added thereto. This solvent frees the carbon of the tar from the soluble constituents thereof, the carbon particles being then held in suspension in the resulting solution.

The next step in the process consists in adding to the mass of the liquid tar an oil of comparatively high hydrocarbon content. The oils I have used have a relatively high viscosity and are much more greasy in character than the light oils used as a solvent. I have employed common fuel oil, gasoline, turpentine, kerosene, and many other such fluids, all of which have proven satisfactory. Common fuel oil and kerosene being the cheapest of those available on the market, are obviously preferable.

This oil when added to the heated liquid causes it to curdle. This curdling of the liquid is a combined chemical and physical action which causes coagulation of the liquid and rapid precipitation of the carbon particles together with a small proportion

of impurities, such as the less readily soluble resins and gums. The resultant coagulum sinks to the bottom of the container whereas the oil and solvent rise to the top. 5 The amount of oil added to the fluid should be sufficient to obtain the maximum amount of coagulated matter from the liquid. That is to say, oil should be added to the liquid until no more coagulation takes place.

10 The next step in the process consists in pouring off the oily fluid from the top of the residue in the bottom of the container. The remaining residue or coagulum is of a brownish tint and is the matter from which 15 I procure carbon.

Now, the next step in the process consists in removing the brown color from the residue. In other words, it is necessary, in order to obtain relatively pure carbon or 20 lamp black that the aforementioned residue be thoroughly washed. I find that this brown color and other impurities may be washed from the residue by adding solvent thereto. The solvent used for this purpose 25 is a product obtained in the manufacture of water gas. This product is obtained by scrubbing the water gas and contains toluol, benzol, and other solvents, being known commercially as light oil. From time to 30 time a sample of the matter may be removed from the liquid and tested to determine if all of the brown matter has been removed therefrom. The test I employed was the usual test for carbon, namely, the white 35 lead test. That is to say, when all of the brown matter has been removed from the residue, the test will give a gray color. I desire it understood also that the solvent employed for purifying the coagulum, may 40 be of any suitable type or kind, though I preferably use light oil as previously mentioned.

The last step in the process consists in pouring off the solvent and drying the carbon or lamp black. Any suitable drying 45 apparatus may be employed.

By employing the above method in manufacturing lamp black from coal tar or water gas tar, I find that about two-thirds of the tar used may be converted into lamp black. 50 In other words, for every pound of tar, I am able to obtain two-thirds of a pound of lamp black. This by far exceeds the amount obtained from tar heretofore.

55 Obviously the solvents employed may be recovered by any suitable distilling process and used over again.

It should be understood, however, that my invention is not to be limited to the 60 exact procedure above described, but only insofar as defined by the scope and spirit of the appended claim.

I claim:

65 The process of producing carbon from tar, which consists in liquefying the tar by

heating it, adding to the liquefied tar a solvent such as benzol, adding to the resulting mixture a relatively heavy hydrocarbon in proper quantity to cause precipitation of the carbon particles of the mixture, removing the precipitate and treating it with a solvent such as light oil and thereby removing the soluble constituents therefrom so as to produce a residuum of substantially pure carbon, and then separating the solvent 75 from the residuum of carbon and drying the latter.

In witness whereof, I hereunto subscribe my name this 18th day of April, 1925.

ALEXANDER L. ULLRICH.

70

75

80

85

90

95

100

105

110

115

120

125

130